

1

3,192,163

### PROCESS FOR THE STABILIZATION OF PETROLEUM LUBRICANTS

Edward B. Hodge, Terre Haute, Ind., assignor to Commercial Solvents Corporation, New York, N.Y., a corporation of Maryland

No Drawing. Filed Mar. 20, 1961, Ser. No. 96,676

19 Claims. (Cl. 252—49.5)

My invention relates to a stabilized petroleum lubricant and more particularly to a process for the production of stabilized petroleum lubricants containing as the active stabilizing agent nitroamines having the structural formula:



where R is lower alkyl and hydrogen and where R<sub>1</sub> is selected from the group consisting of the radical —N(R<sub>2</sub>)<sub>2</sub>, the morpholino radical and the piperidyl radical and R<sub>2</sub> is selected from the group consisting of lower alkyl, lower hydroxyl alkyl, and hydrogen.

It is well known that organisms from the groups consisting of *Corynebacterium*, *Achromobacter*, *Pseudomonas*, *Nocardia* and *Mycobacterium* metabolize petroleum hydrocarbons and fatty acids and thereby produce undesirable oxidation products.

The petroleum industry has long been interested in the stabilization of various petroleum products such as cutting oils, hydraulic fluids, etc., against breakdown by bacteria which metabolize the hydrocarbons with the concurrent formation of deleterious metabolites.

Many compounds have been used as stabilization agents in lubricants, but very few have been found to be commercially successful due to the fact that the compounds are unstable, or are not active against a wide variety of microorganisms.

Among the nitroamines having the above structural formula are included 2-nitro-2-methyl-1,3-bis(dibutylamino)propane, 2-nitro-2-methyl-1,3-bis(2-hydroxypropyl)aminopropane, 2-nitro-2-methyl-1,3-dimorpholinopropane, 2-nitro-2-methyl-1,3-dipiperidylpropane, and 2-nitro-2-ethyl-1,3-bis(dimethylamino)propane. I have found that in some instances I can obtain total inhibition of bacterial growth in petroleum lubricants at concentrations as low as 100 p.p.m. I prefer to include at least 1,000 p.p.m. in most petroleum formulations. However, I can employ amounts up to about 2% by weight of the active nitroamines when the latter is soluble to this extent in the particular petroleum hydrocarbon composition.

I have found that my active ingredients are effective bacteriostatic agents in petroleum containing lubricants such as cutting oils, penetrating oils, grinding lubricants, iron tinning lubricants, core oils, hydraulic fluids, etc.

The following examples set out lubricating compositions in which my active ingredients act as effective bacteriostatic agents. It is not intended that my invention be limited to the compositions, portions, or lubricants set out below; but rather I intend for all equivalents and variations obvious to those skilled in the art to be included within the scope of this specification and the attached claims.

#### Example I

To test the use of my active ingredients in cutting oils, a 25:1 water-cutting oil emulsion was prepared. The cutting oil concentrate used was a proprietary cutting oil containing no bacterial inhibitors sold by Texaco Incorporated under the name of Soluble Oil Texaco-C. To each of one-gallon containers was added 1 liter of water-cutting oil emulsion. Desired amounts of my nitroamines

2

were added to the cutting-oil emulsion in the first container. No inhibitor was added to the other container which was used as a control. At the beginning of the experiment, each unit was inoculated with 5 mls. of a heterogeneous bacterial culture which had grown for several years in a water-cutting oil emulsion. Aeration and mixing were obtained by using an air lift to continually circulate the mixture. The test was continued for a period of six weeks and during the six-week period, 5 mls. of bacterial culture were added at periodic weekly intervals.

The following table sets out the results of the above tests and the number of days of bacterial inhibition when the described concentration of the desired nitroamines were incorporated into the cutting-oil emulsion.

Table I

|    | Nitroamine                                    | Concentration in 25:1 water-cutting oil emulsion | Number of days effective |
|----|-----------------------------------------------|--------------------------------------------------|--------------------------|
| 20 | 2-nitro-2-ethyl-1,3-bis(dimethylamino)propane | 1,000                                            | >42                      |
|    |                                               | 500                                              | 30                       |
|    |                                               | 250                                              | 14                       |
| 25 | 2-nitro-2-methyl-1,3-dimorpholinopropane      | 1,000                                            | >42                      |
|    |                                               | 500                                              | >42                      |
|    | 2-nitro-2-methyl-1,3-dipiperidylpropane       | 1,000                                            | >42                      |
|    | Control                                       |                                                  | 0                        |

30

#### Example II

The following is a water emulsifiable cutting oil which is adequately protected by 1,000 p.p.m. of my nitroamine inhibitors:

|                   | Percent by weight |
|-------------------|-------------------|
| Light mineral oil | 90                |
| Oleic acid        | 10                |

40

The following is a stabilized steam cylinder oil which is adequately protected by 1,000 p.p.m. of 2-nitro-2-methyl-1,3-bis(dimethylamino)propane.

|                        | Percent by weight |
|------------------------|-------------------|
| S.A.E. lubricating oil | 90                |
| Oleic acid             | 10                |

45

The following is a core oil which is adequately protected by 1,000 p.p.m. of 2-nitro-2-methyl-1,3-bis(2-hydroxypropyl)aminopropane.

|                                     | Percent by weight |
|-------------------------------------|-------------------|
| Crude tall oil                      | 25                |
| Fuel oil                            | 35                |
| Tall oil ester (glycol or glycerol) | 40                |

55

#### Example IV

The following is a cutting oil which is adequately protected by 1,000 p.p.m. of 2-nitro-2-ethyl-1,3-bis(dimethylamino)propane.

|              | Percent by weight |
|--------------|-------------------|
| Tallow       | 65                |
| Paraffin wax | 29                |
| Beeswax      | 1.3               |

60

Oxalic acid

Potassium citrate

Urea

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

Percent by weight

metabolizing bacteria, said nitroamine having the structural formula:



5

wherein R is lower alkyl and hydrogen and wherein R<sub>1</sub> is selected from the group consisting of the radical —N(R<sub>2</sub>)<sub>2</sub>, the morpholino radical and the piperidyl radical and R<sub>2</sub> is selected from the group consisting of lower alkyl, lower hydroxyl alkyl, and hydrogen.

2. A liquid petroleum lubricant composition consisting essentially of a liquid petroleum lubricant and a sufficient amount of 2-nitro-2-ethyl-1,3-bis(dimethylamino)propane to stabilize said lubricant against metabolizing bacteria.

3. A liquid petroleum lubricant composition consisting essentially of a liquid petroleum lubricant and a sufficient amount of 2-nitro-2-methyl-1,3-bis(dibutylamino)propane to stabilize said lubricant against metabolizing bacteria.

4. A liquid petroleum lubricant composition consisting essentially of a liquid petroleum lubricant and a sufficient amount of 2-nitro-2-methyl-1,3-dimorpholinopropane to stabilize said lubricant against metabolizing bacteria.

5. A liquid petroleum lubricant composition consisting essentially of a liquid petroleum lubricant and a sufficient amount of 2-nitro-2-methyl-1,3-bis(2-hydroxypropyl) aminopropane to stabilize said lubricant against metabolizing bacteria.

6. A liquid petroleum lubricant composition consisting essentially of a liquid petroleum lubricant and a sufficient amount of 2-nitro-2-methyl-1,3-dipiperidylpropane to stabilize said lubricant against metabolizing bacteria.

7. An aqueous petroleum emulsion consisting essentially of an aqueous petroleum lubricant emulsion and a

sufficient amount of a nitroamine to stabilize said lubricant against metabolizing bacteria, said nitroamine having the structural formula:



10

wherein R is lower alkyl and hydrogen and wherein R<sub>1</sub> is selected from the group consisting of the radical —N(R<sub>2</sub>)<sub>2</sub>, the morpholino radical and the piperidyl radical and R<sub>2</sub> is selected from the group consisting of lower alkyl, lower hydroxyl alkyl, and hydrogen.

15 8. The composition of claim 7 wherein the concentration of the nitroamine is at least 1000 p.p.m. and sufficient to stabilize the lubricant against metabolizing bacteria.

9. The composition of claim 8 wherein the petroleum lubricant is a cutting oil.

10. The composition of claim 9 wherein the petroleum lubricant is a steam cylinder oil.

#### References Cited by the Examiner

#### UNITED STATES PATENTS

|    |           |       |         |           |
|----|-----------|-------|---------|-----------|
| 25 | 2,381,408 | 8/45  | Senkus  | 167—22 XR |
|    | 2,474,791 | 6/49  | Senkus  | 260—247   |
|    | 2,913,414 | 11/59 | Hodge   | 252—51.5  |
|    | 2,976,244 | 3/61  | Bennett | 252—51.5  |
|    | 2,987,479 | 6/61  | Bennett | 252—51.5  |
|    | 3,054,748 | 9/62  | Hodge   | 167—22    |

DANIEL E. WYMAN, Primary Examiner.

JULIUS GREENWALD, ALPHONSO D. SULLIVAN,  
Examiners.